

Patented Oct. 13, 1953

2,655,477

# UNITED STATES PATENT OFFICE

2,655,477

## MINERAL LUBRICATING OIL CONTAINING AN ANTICORROSION AGENT AND AN ANTI- OXIDANT DETERGENT AGENT

John D. Bartleson, Cleveland, and Milton H. Campbell, Cleveland Heights, Ohio, assignors to The Standard Oil Company, Cleveland, Ohio, a corporation of Ohio

No Drawing. Application December 27, 1946,  
Serial No. 718,890

1 Claim. (Cl. 252—32.7)

**I** This invention relates to lubricants, and more particularly to lubricating oils containing both a detergent type agent and a reaction product of phosphorus sulfide and an olefin as an anti-deterioration agent. These oils are relatively non-corrosive and non-lacquer forming.

Such lubricants are suitable for use under various conditions, including high temperatures or high pressures or both, as for instance, use in an internal combustion engine operating at high temperatures and in which the lubricant is in close contact with metallic surfaces, metal compounds and high temperature gases.

The art appreciates that many diverse factors are involved in attaining a single lubricating oil addition agent which imparts to the oil little or no lacquer formation and also shows little or no deterioration or corrosion of metals, especially bearing metals with which the lubricant comes in contact, as well as low oxidative deterioration, as indicated by low viscosity increase, sludge, etc. It is very difficult to produce a single addition agent which is nearly optimum for all these factors, especially at a commercially interesting cost.

Another approach to the problem of producing a lubricating oil which shows little or no lacquer deposition and little or no corrosion of metals, especially bearing metals with which the lubricant comes in contact, as well as little or no oxidative deterioration, is to use two or more addition agents with the lubricating oil, each agent imparting at least one of the desired characteristics, viz.: anti-lacquer, anti-corrosion, anti-oxidant, to the oil. In this approach, the effect of the addition agents upon each other comes into play, and the undesirable characteristic imparted by one agent may more than overcome the desirable effects of another agent as to this characteristic. For instance, many anti-lacquer or detergent-type agents impart to a lubricating oil a non-lacquer forming characteristic, but at the same time greatly increase the normal corrosion characteristic of the oil. Thus, any anti-corrosion agent which is blended therewith must overcome the corrosion imparted by the anti-lacquer agent as well as the corrosion characteristic of the oil base stock itself. It must also not interfere with the anti-lacquer effect of the first agent if the lubricant is to have optimum anti-corrosion as well as anti-lacquering characteristics. If a third blending agent is required to impart other anti-oxidant characteristics, it is evident that these factors or inter-

**2** effects of the agents on each other, as well as on the oil, will be increased manifold times.

Further difficulties which are encountered include the harmful effect of one agent upon the desired characteristic imparted to the oil by another agent, thus neutralizing the desirable effect imparted by the latter. Many of the presently known corrosion inhibitors function as corrosion inhibitors because they form a film of lacquer which protects the metal parts. Thus it would be expected that a good corrosion inhibitor would give a very poor varnish rating. Furthermore, it would be expected that a detergent which is strong enough to remove varnish formed on the pistons due to the presence of the anti-corrosion additive, would also remove the protective film on the bearings, thus obviating the beneficial effect of the corrosion inhibitor. Such has been the case with many anti-corrosion additives. For instance, a small amount of p,p-di-(dimethylamine)-diphenylmethane satisfactorily decreases the corrosion characteristics of a conventional solvent extracted oil containing a small amount of the barium derivative of the reaction product of dioctadecylamine with P<sub>2</sub>S<sub>5</sub>. However, in so doing, it lowers the piston skirt rating to an unacceptable value. It is very difficult, if not impossible, to predict beforehand the characteristics of a lubricating oil containing two or more addition agents from the characteristics imparted by each agent alone.

It has been found that an agent having anti-deterioration (anti-corrosion or anti-oxidation or both) properties may be prepared by reacting a phosphorus sulfide with a lower olefin having a sufficiently high molecular weight to give an oil-soluble reaction product. However, a lubricating oil containing this agent, e. g., about 1.5 per cent by weight thereof, is very unsatisfactory as to lacquer and sludge characteristics. The overall rating characteristic of an oil with the agent is also very low.

In accordance with the invention, it has been found, and quite surprisingly, that an anti-lacquer or detergent type agent may be added to a lubricating oil composition together with the above described anti-deterioration agent and the resulting blend will have substantially the desirable non-lacquering characteristics imparted by the detergent-type agent plus substantially the desirable anti-deterioration characteristics imparted by the phosphorus sulfide-olefin anti-deterioration agent; that the undesirable corrosion characteristics due to the oil or the oil plus the anti-lacquer agent are overcome by the anti-cor-

3

rosion agent; and that the very bad lacquer characteristic due to the anti-corrosion agent as well as that of the oil are completely overcome by the anti-lacquer agent. The presence of the phosphorus sulfide-olefin additive does not detract from the desirable anti-lacquer characteristic imparted to the oil by the detergent-type agent, and likewise the detergent-type agent does not detract from the desirable anti-corrosion characteristic imparted by the phosphorus sulfide-olefin agent.

This discovery is of especial commercial significance in view of the relatively low cost of the phosphorus sulfide-olefin type agent and some of the more efficient metal type anti-lacquering agents (which are very corrosive, however), as well as the ease with which the blends may be prepared.

The objects achieved in accordance with the invention include the provision of a blend of agents which blend may be useful itself as a lubricant and which when blended in lubricating oils will markedly improve the lacquer, sludge, corrosion and other characteristics thereof; the provision of relatively non-lacquering and non-deteriorative lubricating oils containing such agents; and other objects which will be apparent as details or embodiments of the invention are set forth hereinafter.

#### The detergent type agents

The detergent type agents which may be used contain one or more of an alkali metal, such as sodium, potassium and lithium, or an alkaline earth metal, such as calcium, barium and strontium. They may be illustrated by an alkali or alkaline earth metal derivative of a reaction product of phosphorus pentasulfide with an amine, such as dioctadecylamine or octadecenylamine. These neutralized phosphorus pentasulfide derived agents impart certain anti-oxidant characteristics to the blend, also. They impart to the oil the undesirable characteristic of corroding metals, especially the bearing metals with which the lubricant contacts.

The amount of the detergent type agent usually added to the oil or grease depends upon the characteristics of the oil or grease and the intended use, as known to the art, and in general ranges from a fraction of one per cent up to about ten per cent.

#### The anti-deterioration agent

The anti-deterioration agent employed in accordance with the invention is a phosphorus sulfide-olefin reaction product which may be made with direct admixture of the reactants, or, if desired, by their admixture in the presence of a diluent which may or may not be subsequently removed. A heavy oil such as white oil, or a lubricating oil having about the same properties as that to which the new composition is to be added may be used as a diluent. The reaction is usually complete in about 10 hours or less time. The reaction time is a function of the temperature, the amount of the sulfide that is to react, the subdivision of the reactants, the rate of stirring, etc.

The olefin or mixture of olefin may be reacted with the phosphorus sulfide or a mixture of phosphorus sulfide in weight ratios from 5 to about 95 weight per cent of the phosphorus sulfide based on the weight of the olefin, depending on the molecular weight of the olefins used. Generally about 25 to about 75 per cent is the usual range that will be used, and about 50 to about 70 per cent.

cent is especially desirable. Even small amounts show a significant improvement, and economic factors would make it undesirable to use more than is necessary to achieve the desired improvement.

Phosphorus pentasulfide is prepared although other phosphorus sulfides or mixtures of sulfides may be employed. Phosphorus pentasulfide is most economic and readily available and for this reason is used in the illustrative examples. Under suitable conditions sulfides of arsenic or antimony may be similarly employed.

In general, olefins having from about 6 to about 25 carbon atoms in the molecule are preferred. A commercially desirable olefin is so-called "motor polymer" or "reduced motor polymer." Motor polymer is usually made from C<sub>3</sub> and C<sub>4</sub> olefins by non-selective polymerization, e. g., with a phosphorus acid type catalyst. A polymer gasoline fraction may be removed therefrom by fractional distillation to the 250° F. cut point, and the residue is known as "reduced motor polymer." The reduced motor polymer may contain small amounts of materials lighter than the trimer. Its average molecular weight is about 145 and it preferably contains a major amount of olefins boiling below 600° F. The olefins used should be of a sufficiently high molecular weight to give a final product having the desired oil dispersibility.

The reaction may be carried out in the presence or absence of air, or in an atmosphere of inert or non-deleterious gas, such as nitrogen or H<sub>2</sub>S. It may also be carried out under pressure, e. g., the pressure generated when the reaction is carried out in a closed vessel.

The yield is very high and appreciable amounts of oil insoluble products are not formed. Generally the amount of sulfide is chosen so that all of it will react at the temperature selected and the reaction is continued until it is consumed.

After the reaction is complete, the sulfide-olefin reaction product is suitable for use as an anti-corrosion addition agent, but preferably it is first processed, for instance, centrifuged or filtered, to remove water and any traces of oil-insoluble by-product substances.

The amount of the sulfide-olefin to be incorporated in the oil or grease, together with the anti-lacquer detergent type agent, will also depend upon the intended use as well as the characteristics of the oil or grease, and in general, amounts in the range of from 0.02 per cent to 2.0 per cent by weight, based on the oil, are suitable. Even small amounts show a significant improvement and it is uneconomical to add more than is necessary to impart to the lubricant the desired properties.

The following examples or tests of lubricant compositions, prepared in accordance with the invention, will serve to illustrate and point out some advantages but in no wise to limit the scope of the invention as otherwise disclosed and claimed herein.

#### EXAMPLE 1

##### Anti-corrosion addition agent

806 grams of reduced motor polymer and 494 grams of phosphorus pentasulfide were mixed and heated in a closed vessel at 350° F. for 8 hours, with agitation. The reaction mass was then filtered hot. The filtrate was used as the agent of Example 1 in the tests reported hereinafter.

## EXAMPLE 2

## Anti-lacquer addition agent

The barium derivative of the reaction product of phosphorus pentasulfide with dioctadecylamine was prepared in accordance with known procedures by reacting phosphorus pentasulfide with the amine and then treating the reaction product with barium hydroxide octahydrate (see U. S. Patent No. 2,403,894). This is the addition agent of Example 2 used in the tests referred to hereinafter, in conjunction with the sulfide-olefin anti-corrosion blending agent.

In testing the oils containing the addition agents the so-called standardized "Chevrolet Engine Test" was used. In this test, new piston rings and two new copper-lead bearing inserts are installed in the motor prior to each test. The engine is a conventional Chevrolet engine with 216.5 cu. in. piston displacement and a compression ratio of 6.5 to 1. The engine is operated at 3150 R. P. M. with a load of 30 B. H. P. and at a temperature at the jacket outlet of 200° F. The lubricating oil temperature is maintained at 265° F. for an SAE 10 grade oil, and at 280° F. for oils of SAE 30 to 50 grades. The fuel used contains from 2.5 to 3.0 ml. tetraethyl lead per gallon. Besides the weight loss of the test bearings, deposits in the power section, and properties of the used oil, sampled near the middle and also at the end of the test, are examined.

A conventional solvent extracted lubricating oil base stock (SAE 30) and blended compositions of this oil made in accordance with the invention were submitted to 36-hour tests in accordance with the above Chevrolet engine procedure. The results in the following table are typical.

TABLE I

| Column No.                                                                  | 1     | 2     | 3     | 4     | 5     |
|-----------------------------------------------------------------------------|-------|-------|-------|-------|-------|
| Concentration of Example 1 (anti-corrosion) agent in percent by weight      | 0     | 1.5   | 0     | 0.19  | 0.38  |
| Concentration of Example 2 (anti-lacquer) agent in percent by weight        | 0     | 0     | 2.0   | 2.0   | 2.0   |
| Piston skirt rating                                                         | 9.50  | 6.25  | 9.75  | 9.75  | 9.75  |
| Varnish rating                                                              | 48.75 | 43.00 | 49.0  | 49.55 | 49.25 |
| Sludge rating                                                               | 43.25 | 42.25 | 49.25 | 48.50 | 48.0  |
| Overall rating                                                              | 92.00 | 85.25 | 98.25 | 98.05 | 97.25 |
| Corrosion of Cu-Pb bearing metal (in mgms. wt. loss per bearing half-shell) | 1.428 | 8     | 417   | 169   | 79    |
| Viscosity increase                                                          | 210   | 136   | 189   | 162   | 168   |
| Pentane insolubles (mgms.)                                                  | 110   | 184   | 44    | 54    | 27    |

Column 3 shows that the anti-lacquer agent has excellent piston skirt, varnish, sludge and overall ratings, but the corrosion is bad. One would expect these excellent ratings to be brought down by the addition to the anti-lacquer agent of the sulfide-olefin anti-corrosion agent, in view of the data in column 2 showing low piston skirt, varnish, sludge and overall ratings for the latter agent.

Column 4 and column 5 of the above table, however, show that in blends containing the anti-lacquer agent and also the anti-corrosion agent, in accordance with the invention, the varnish rating is even slightly better than that of the blend containing the anti-lacquer agent alone (column 3). The sludge rating and overall rating are substantially equivalent to those of the oil blend containing only the anti-lacquer agent (column 3). The great improvement in the corrosion characteristics is particularly noteworthy, especially in view of the excellent var-

nish, sludge and overall rating of the blends containing the two agents, in accordance with the invention. Furthermore, the viscosity increase rating is improved somewhat, and the pentane insolubles are desirably low for the combination blends.

The piston skirt rating remained high throughout the test of the blend containing 0.38 per cent of the anti-corrosion agent (column 5) and was 9.5 after the test was extended to 72 hours. Even after the 72-hour test the oil was substantially unoxidized, as indicated by testing the used oil. This is remarkable in view of the high anti-lacquer characteristics and low corrosion characteristics of the lubricant blend prepared in accordance with the invention.

The blend made in accordance with the invention was also tested by the Caterpillar 96-hour single-cylinder 4-cycle diesel engine test which was developed several years ago as a shortened version of the standard 480-hour Caterpillar 1-A test (CRC-L-1). It is of considerable value in predicting the performance of an oil in the standard test, although it is somewhat more severe than the latter. The purpose of the 96-hour test is to determine the effect of lubricating oils on ring sticking, wear, and the accumulation of deposits in a single cylinder 4-cycle diesel engine having a standard crankcase designed with minimum recesses or pockets to retain oil, a cylinder bore of 5.75 in., a stroke of 8 in. and a piston displacement of 208 cu. in. The engine is operated at about 1000 R. P. M. under a load of 19.8 B. H. P. for a fuel input of about 3000 B. t. u. per minute for 96 hours (continuously, if possible), with an inlet cooling jacket temperature of about 185° F. and an outlet temperature of about 195° F. The temperature of the oil going to the bearings is about 195° F., the air inlet temperature is about 95° F., and the oil pressure at the bearings is 30 p. s. i. At the end of the 96-hour test the liner, piston, rings, crankcase, and engine parts are completely inspected with respect to low carbonaceous deposits, resistance to ring sticking and resistance to scratching. The liner is measured both before and after the test. The maximum wear is recorded as the difference between the initial and final readings. The maximum and minimum top ring side clearance is observed both before and after the test, and is recorded. The oil filter element is completely inspected at the end of the 96-hour test as to quantity and type of sludge deposits. The results are reported on a numerical rating system similar to the U. S. Navy Department Demerit System. The individual engine parts or items are first evaluated by means of a demerit system which is designed to minimize personal evaluation and judgment in the inspection of conditions chargeable to the lubricant. Demerits for each item are then justified by weighting factors which closely establish the relative importance of the engine factors involved. The weighted demerits are totalled and subtracted from 100 for the final or merit rating.

## A. Engine cleanliness

The initial ratings are made in accordance with a demerit system. The deposits on various engine parts, as listed in the following tabulations, are evaluated between the demerit range of 0, a clean engine part, and 10, the maximum depositions. The relative importance of the de-

7  
posits in regard to engine performance is reflected by the weighting factor involved.

|                                                | Possible basic demerits | Weighting factor | Possible weighted demerits |
|------------------------------------------------|-------------------------|------------------|----------------------------|
| 1. Ring sticking                               | 10                      | 2.0              | 20                         |
| 2. Liner deposits (cylinder above ring travel) | 10                      | 1.0              | 10                         |
| 3. Crosshead lacquer (skirt deposit)           | 10                      | 1.5              | 15                         |
| 4. Heat groove deposit (top land)              | 10                      | 1.0              | 10                         |
| 5. Ring groove deposits                        | 10                      | 2.0              | 20                         |
| 6. Piston land deposits                        | 10                      | 2.0              | 20                         |
| 7. Oil system sludge deposits                  | 10                      | .5               | 5                          |
| Total possible weighted demerits               |                         |                  | 100                        |

<sup>1</sup> The rating of this item is not possible when standard "L-1" 430-hr. piston (KX7288) is employed. Therefore, the total weighted demerits is divided by 90 to convert the final rating to a 100 basis when this item is not included in the rating.

### B. Overall wear

The initial ratings are made in accordance with a demerit system. When no measurable wear of the piston rings and liner or scuffing of the piston is evidenced, the demerit value is scored as 0. When the assigned limits of wear and scuffing (itemized below) are exceeded, the demerit value becomes 10. Intermediate values are judged accordingly. The final rating is computed from the following three factors which are adjusted by weighting factors in accordance with their relative importance in the test:

|                                     | Possible basic demerits | Weighting factor | Possible weighted demerits |
|-------------------------------------|-------------------------|------------------|----------------------------|
| 1. Cylinder liner wear              | 10                      | 4.0              | 40                         |
| 2. Compression ring wear            | 10                      | 2.0              | 20                         |
| 3. Piston scuffing (above top ring) | 10                      | 4.0              | 40                         |
| Total possible weighted demerits    |                         |                  | 100                        |

A blend of conventional solvent extracted Mid-Continent lubricating oil base stock (SAE 30) containing 0.38% by weight of the anti-corrosion agent of Example 1, and 1.5% by weight of the anti-lacquer agent of Example 2, based on the oil, was tested in accordance with the above Caterpillar 96-hour procedure and the following results were obtained.

|                       | Possible demerits | Actual demerits |
|-----------------------|-------------------|-----------------|
| Ring sticking         | 20                | 0               |
| Liner deposits        | 10                | 2.9             |
| Skirt deposit         | 15                | 1.2             |
| Heat groove deposit   | 10                | 1.7             |
| Ring groove deposit   | 20                | 1.2             |
| Piston land deposits  | 20                | .8              |
| Oil system sludge     | 5                 | .05             |
| Total demerits        | 100               | 5.85            |
| Cylinder liner wear   | 40                | 2.0             |
| Compression ring wear | 20                | 2.6             |
| Piston scuffing       | 40                | 12              |
| Total                 | 100               | 16.6            |

It is evident from the foregoing table that the oil blend made in accordance with the invention shows a very high merit rating.

The Sohio corrosion test was used in evaluating other blends made in accordance with the invention. This test is described in U. S. Patent No. 2,464,233, dated March 15, 1949, to E. C. Hughes, J. D. Bartleson, M. L. Sunday and M. M. Fink, which also correlates the results of the laboratory tests with a Chevrolet engine test. Essentially the laboratory test equipment con-

5  
sists of a vertical thermostatically heated glass test tube (45 mm. outside diameter and 42 cm. long) into which is placed the corrosion test unit. An air inlet is provided for admitting air into the lower end of the corrosion unit in such a way that in rising the air will cause the oil and suspended material therein to circulate into the corrosion unit. The tube is filled with an amount of the oil to be tested which is at least sufficient to submerge the metals being tested.

10  
The corrosion test unit essentially consists in a circular relatively fine grained copper-lead test piece of  $1\frac{1}{8}$ " O. D., which has a  $\frac{1}{4}$ " diameter hole in its center (i. e. shaped like an ordinary washer). The test piece has an exposed copper-lead surface of 3.00 sq. cm. Of this surface area, 1.85 sq. cm. acts as a loaded bearing, and is contacted by a part of the cylindrical surface of a hardened steel drill rod ( $\frac{1}{4}$ " diameter  $\frac{31}{32}$ " long, and of 51-57 Rockwell hardness).

20  
The drill rod is held in a special holder, and the holder is rotated so that the surface of the drill rod which contacts the bearing sweeps the bearing surface (the drill rod is not rotated on its own axis and the surface of the drill rod which contacts the bearing is not changed).

25  
The corrosion test unit means for holding the bearing and the drill rod is a steel tubing (15" long and  $1\frac{1}{2}$ " O. D.) which is attached to a support. A steel cup (1" long,  $1\frac{1}{2}$ " O. D. by  $1\frac{1}{8}$ " I. D.) is threaded into the steel tube, at the lower end. The cup has a  $\frac{1}{8}$ " diameter hole in the bottom for admitting the oil into the corrosion chamber. The copper-lead test piece 30 fits snugly into the steel cup and the hole in the test piece fits over the hole in the steel cup. A section of steel rod ( $\frac{3}{8}$ " in diameter and 19" long) serves as a shaft and is positioned by 2 bearings which are fixedly set in the outer steel tubing, one near the top and one near the lower (threaded) end thereof. Several holes are drilled just above and just below the lower bearing. The holes above the bearing facilitate cleaning the apparatus, while the holes below the bearing enable the circulation of oil through the corrosion chamber. The drill rod holder is connected to the shaft by a self-aligning yoke and pin coupling. This assures instantaneous and continuous alignment of the drill rod bearing member against the bearing surface at all times.

35  
50  
A pulley is fitted to the top of the steel shaft and the shaft is connected therethrough to a power source. The shaft is rotated at about 675 R. P. M.; and the weight of the shaft and attached members is about 600 grams, which is the gravitational force which represents the thrust on the bearing. The air lift from the air inlet pumps the oil through the chamber containing the test piece and out through the holes in the steel tubing.

55  
60  
65  
The ratios of surface active metals to the volume of oil in an internal combustion test engine are nearly quantitatively duplicated in the test equipment. The temperature used is approximately that of the bearing surface. The rate of air flow per volume of oil is adjusted to the same as the average for a test engine in operation. Of the catalytic effects, those due to soluble iron are the most important. They are empirically duplicated by the addition of a soluble iron salt. Those due to lead-bromide are duplicated by its addition.

70  
75  
The test was correlated with a slightly modified version of the L-4 Chevrolet test. This modification comprised reducing the oil addi-

tions from the 4 quarts in the usual procedure to 2 quarts, by reducing the usual 1 pint oil additions which are made at 4 hour intervals to  $\frac{1}{2}$  pint additions. This modification increases the severity of the test in its corrosion and detergency components, particularly in the case of border line oils.

For each test, the glass parts are cleaned by the usual chromic acid method, rinsed and dried. The metal parts are washed with chloroform and carbon disulfide and polished with No. 925 emery cloth or steel wool. A new copper-lead test piece is used for every test. The test piece is polished before use, on a surface grinder to give it a smooth finish. The test piece is weighed before and after the test on an analytical balance to evaluate the corrosion. After placing the oil and corrosion test unit in the tube, and bringing the assembly up to temperature in the thermostat, soluble catalyst is added and the air flow is started. Lead bromide catalyst is added immediately after starting the air, and timing of the test is begun.

The laboratory test conditions which were found to correlate with the modified Chevrolet procedure 36-hour test are shown in the following table.

TABLE A

|                   |                                                                                 |
|-------------------|---------------------------------------------------------------------------------|
| Temperature       | 325° F.                                                                         |
| Oil sample        | 107 cc.                                                                         |
| Air flow rate     | 70 liters/hour.                                                                 |
| Time              | 10 hours.                                                                       |
| Catalysts         | Steel.                                                                          |
|                   | Copper-lead bearing: 3 sq. cm. area of which 1.85 sq. cm. is a bearing surface. |
|                   | Ferric 2-ethyl hexoate: 0.05% as $\text{Fe}_2\text{O}_3$ in C. P. benzene.      |
|                   | Lead bromide: 0.1% as precipitated powder.                                      |
| Bearing assembly: |                                                                                 |
| Load              | 600 grams.                                                                      |
| Speed             | 675 R. P. M.                                                                    |

By extending the laboratory test to 20 hours, it was found that correlation with the modified Chevrolet 72-hour test could be obtained.

At the close of the test period, the extent of corrosion is determined by reweighing the corrosion test piece and determining the change in weight due to the test. An accurate evaluation of the lacquering properties of an oil is obtained by a visual rating system which is applied to the outer surface of the corrosion unit steel tube and metal cup in much the same way that the piston skirt, cylinder wall, etc. of an engine are rated for varnishes. The sludge rating of the engine is simulated by a visual rating of the insoluble materials and used oil which are coated on the glass test tube at the conclusion of the test. For both sludge and varnish rating a scale rating of A (best) to F (worst) is used.

A sufficient volume of used oil is obtained from the test for determination of the usual used oil properties, such as pentane insolubles, viscosity increase, and neutralization number.

## EXAMPLE 3

The potassium derivative of the reaction product 70 of phosphorus pentasulfide with an unsaturated amine

A commercially available unsaturated primary amine mixture containing about 80 per cent by 75

## 10

weight of octadecenyl and octadecadienyl radicals and about 20 per cent of hexadecenyl radicals was used in the following preparation. This amine contained about 1.25 olefinic double bonds per molecule of amine, as an overall average, and had an iodine number in the range of 100 to 110.

810 grams of the above unsaturated amine and 330 grams of phosphorus pentasulfide were mixed with 2430 grams of lube oil, as a diluent, and heated at 500° F. for thirty minutes, with agitation. The resulting reaction mass was filtered hot. After filtering, the product was mixed with 38.4 grams of added sulfur, and the mixture heated, whereby the filtrate was sulfurized.

3413 grams of this sulfurized filtrate and 202 grams of potassium hydroxide and 388 grams of water were mixed and heated with agitation at 190° F. for three hours. The reaction mass was blown with air while maintained at 250° F. for 20 two hours. It was then filtered hot. This is the anti-lacquer agent in Table II in the tests reported hereinafter.

TABLE II

| Column No.                                                                                             | 1             | 2          | 3         |
|--------------------------------------------------------------------------------------------------------|---------------|------------|-----------|
| Anti-corrosion agent of Example 1 concentration in percent by weight (of oil)                          |               |            |           |
| 30 Anti-lacquer agent of example No. Concentration of anti-lacquer agent in percent by weight (of oil) | None          | None       | 0.38      |
| Corrosion of Cu-Pb (in mgms. wt. loss of)                                                              | None          | 1          | 1         |
| Viscosity increase (SUS) Neut. No.                                                                     | 72.1<br>3,930 | 9.9<br>143 | 3.5<br>18 |
| 35 Sludge rating                                                                                       | 7.7           | 1.2        | 0.4       |
|                                                                                                        | A+            | A+         | A+        |

Again, it is evident from the above data that the oil blend containing a phosphorus sulfide derived metal type anti-lacquer agent is further improved as to anti-corrosion and anti-oxidant characteristics by the incorporation of a sulfide-olefin anti-deterioration agent, in accordance with the invention, without impairing the anti-sludge characteristics imparted by the metal type agent.

In order to prevent foaming of the oil containing additives of the invention, it may be desirable in some cases to add a very small amount of tetra-amylosilicate, or an alkyl ortho carbonate, ortho formate or ortho acetate, or polyalkyl-silicone oil.

Variations and modifications of the invention will be apparent to one skilled in the art in view of the foregoing disclosures, and the invention contemplates them broadly except as limited by the appended claim.

We claim:

A mineral oil lubricant comprising a major proportion of mineral lubricating oil and an amount of an anticorrosion agent within the range of about 0.19 to about 0.38% based on the weight of the oil and 2% based on the weight of the oil of an antioxidant detergent agent, said amount of each agent being sufficient to inhibit the development of both corrosion and lacquer when the oil is used under service conditions to a greater extent than the same amount of either agent alone under the same conditions, said anticorrosion agent being an oil-dispersible reaction product of phosphorus pentasulfide and "reduced motor polymer" in the ratio of about 1.5 moles "reduced motor polymer" per mole of phosphorus pentasulfide, formed at about 350° F. for about

eight hours, and said antioxidant detergent agent being an oil-dispersible barium derivative of a reaction product of phosphorus pentasulfide and dioctadecylamine in the ratio of about 1.6 moles dioctadecylamine per mole of phosphorus pentasulfide, formed at about 500° F. for about thirty minutes.

JOHN D. BARTLESON.  
MILTON H. CAMPBELL. 10

References Cited in the file of this patent  
UNITED STATES PATENTS

| Number    | Name         | Date          |
|-----------|--------------|---------------|
| 2,316,078 | Loane et al. | Apr. 6, 1943  |
| 2,316,079 | Loane et al. | Apr. 6, 1943  |
| 2,316,080 | Loane et al. | Apr. 6, 1943  |
| 2,381,907 | Hughes       | Aug. 14, 1945 |
| 2,403,894 | Bartleson    | July 9, 1946  |
| 2,447,607 | Zimmer       | Aug. 24, 1948 |